

J. D. Wise.

Casting Building Blocks.

No. 86,961.

Patented Feb. 10, 1869.

Fig. 1.



Fig. 2.



Fig. 3.



Fig. 5.



Fig. 4.



Witnesses,

R. T. Campbell.  
L. T. Campbell.

Inventor:

John D. Wise  
by  
Mason, Fenwick & Lawrence.

# United States Patent Office.

JOHN D. WISE, OF GERMAN TOWNSHIP, OHIO, ASSIGNOR TO HIMSELF AND CHARLES DEIBOLD, OF THE SAME PLACE.

Letters Patent No. 86,961, dated February 16, 1869.

## IMPROVEMENT IN CASTING BUILDING-BLOCKS.

The Schedule referred to in these Letters Patent and making part of the same.

To all whom it may concern:

Be it known that I, JOHN D. WISE, of German township, Holmes county, and State of Ohio, have invented a Method of Utilizing the Slag of Iron-Furnaces in the Production of Block for Building and other Purposes; and I do hereby declare that the following is a full, clear, and exact description thereof, reference being had to the accompanying drawings, making a part of this specification, in which—

Figure 1 is a perspective view of a moulded block of slag, with one corner broken away, to show the strengthening-band which is moulded in the block.

Figure 2 is a cross-section through the centre of a flask, showing a block of the slag in it, ready to be removed.

Figure 3 is a longitudinal central section through the flask.

Figure 4 is a top view of the flask.

Figure 5 is a perspective view of a strengthening-band, with its supports, and corner-strengthening wires.

Similar letters of reference indicate corresponding parts in the several figures.

The object of this invention is to utilize the slag or waste of iron-furnaces, by moulding the slag into rectangular or other-shaped blocks, suitable for building, paving, and other analogous purposes.

I have discovered that the slag which is drawn from furnaces, in the process of smelting iron-ore, and which has heretofore been thrown away as useless, will, if moulded in proper flasks, produce very hard and durable blocks, which are well adapted for use in the construction of buildings, and for paving-purposes.

The following is a description of one practical mode of moulding the slag into a useful form:

I employ a metal flask, in order that it shall not be seriously injured by the heat to which it is subjected, and construct this flask of four or more plates or sections united together, so that, after a block is moulded within the flask, they can be readily separated, to allow of the removal of the block.

C is the top plate or section, which, in the present instance, is rectangular, with a pouring-hole, c, through its centre, as shown in figs. 2, 3, and 4.

E is the bottom section, which is of the same size and shape as the top section, and which has lugs, or forked offsets, on two of its edges, for receiving and holding the lower ends of two clamping-rods, F F, by which the several sections of the flask are confined in place.

J J' are the perpendicular side plates of the flask, which may be, for convenience, secured permanently together in pairs.

The abutting-surfaces of the several plates or sections may be provided with dowel-pins, fitting in corresponding-holes, so as to make strong and tight joints at the angles of the flask.

To put the sections of the flask together, the side plates J J' are adjusted on top of the bottom plate E, and on top of these side plates the cover C is put.

This cover C has slotted, or forked lugs d e, upon its edges, which, when the plates C and E are in their proper places, are directly over the lugs i i, on plate E.

The rod F, with heads g on both ends, confines one side of the flask-plates, and the opposite bar F, which has a head, g, on its lower end, and a key, f, passed through it, over plate C, confines the other side of the flask. Other means may be adopted for confining the flask-sections together.

Before putting the top plate C on the flask, a narrow band, B, fig. 5, of a rectangular form, and somewhat smaller than the interior chamber of the flask, is adjusted centrally within this chamber, by supporting it upon the bottom of the flask, by means of the vertical wires b b, applied at its four angles.

Figs. 1, 2, and 3, show this band embedded in the body of the casting A, with its upright wires b b, in the four corners of the casting.

If desirable, one or more of the inner surfaces of the flask-plates may have elevations and depressions formed on them, for producing, in converse order, corresponding figures upon the exterior surface or surfaces of the block A, thereby ornamenting the same, as indicated at a, in figs. 1 and 2.

When the flask-sections have been confined together in a proper manner, the flask is taken to the iron-furnace, and, at a suitable time, for drawing off the slag, the furnace is opened at the proper point, and the melted slag run directly into the mould, producing, when cool, a block, A, which is prevented from cracking, while cooling, by the metallic band B, embedded in it, as above shown.

Blocks, thus produced, possess great strength and solidity, and are well adapted for the purposes above named. They have a dark color, and present glazed surfaces, resembling a finely-finished polish. For building-purposes, they may be moulded of any required size and shape; and, if found necessary, the blocks or slabs may be produced with chambers in or through them for receiving mortar, by which to unite the blocks together, in a building.

Having described my invention,

What I claim as new, and desire to secure by Letters Patent, is—

A brick or block made from slag, and stayed and held together by internal devices, substantially as described.

JOHN D. WISE.

Witnesses:

JOHN LUKE,  
FRANCIS LAMBRÉCHT.